

Patented Feb. 16, 1926.

1,572,905

# UNITED STATES PATENT OFFICE.

OTHO V. STEWART, OF WILKINSBURG, PENNSYLVANIA, ASSIGNOR TO WESTINGHOUSE ELECTRIC & MANUFACTURING COMPANY, A CORPORATION OF PENNSYLVANIA.

## IMPREGNATING WOOD.

No Drawing.

Application filed December 16, 1920. Serial No. 431,289.

*To all whom it may concern:*

Be it known that I, OTHO V. STEWART, a citizen of the United States, and a resident of Wilkinsburg, in the county of Allegheny and State of Pennsylvania, have invented a new and useful Improvement in Impregnating Wood, of which the following is a specification.

This invention relates to the impregnating of wood, more especially to the impregnating of wood strain-insulators for use in high-voltage transmission lines.

Such insulators should have relatively great strength, be impervious to moisture, and have excellent insulating properties. The present invention is designed to produce an insulator of the above type, which is very resistant to moisture and to changes in atmospheric conditions, which has great 20 mechanical strength and is an excellent insulator.

In order to produce a strain-insulator of wood having such desirable properties, it has been attempted, at various times, to 25 treat wood sticks by various methods, such as seasoning the wood, boiling or steaming the same, impregnating with various substances, such as gums, oils, or waxes of various kinds under pressure, or at atmospheric pressure, or in a partial or complete 30 vacuum. A favorite method of impregnating has consisted in placing sticks under a vacuum and subjecting the same to heat for a considerable length of time. During this 35 vacuum-and-heat treatment, asphalt was allowed to come in contact with the wood at the elevated temperature in order to impregnate the same. A further treatment, consisting in applying pressure to the 40 heated mass so treated, was then usually employed.

Such processes had many disadvantages in that the gummy or asphaltic material 45 penetrated but slightly below the surface of the wood, rarely ever penetrating more than one-eighth of an inch in depth. Furthermore, these processes were complicated and relatively expensive, since they usually utilized a vacuum or pressure, or both. For this 50 reason, it was generally necessary to treat the material in closed vessels. On account of the viscosity of the asphalt or other similar material used, the impregnation was not uniform and the impregnated wood was, 55 therefore, not uniformly resistant to the tem-

perature and moisture changes in the atmosphere. The interior of the wood was generally not impregnated at all, and, since the impregnation of the surface was not uniform, moisture often entered the interior 60 and caused deterioration of the wood.

In practising my invention, I impregnate the wood, preferably partially dried, with a substance which penetrates easily and is capable of filling all the pores of the wood. 65 This material may be a relatively light substance which melts at a low temperature and has a relatively low boiling point. It is merely necessary that this substance be an insulator and have a low viscosity in order 70 to more readily penetrate the wood. I subsequently treat the wood so impregnated with a heavy non-volatile material which coats the outer portion of the wood, preventing the loss of the first substance which 75 penetrates the entire body of the wood and thus increases the insulating properties thereof and insures the exclusion of moisture therefrom. The substance, which I prefer to use for the first impregnation, is a wax, such as paraffin, and for the second treatment, I prefer to use a gummy material, such as an asphalt.

My new process is preferably carried out 80 as follows: Wood is cut to the proper size and shape and is then kiln-dried until the moisture content is about ten to twelve per cent. The wood is then immersed in a bath of molten paraffin, which is at a temperature generally not exceeding 130° C., for a period 85 of from five to six hours. The wood is removed from the paraffin bath and immersed in a bath of molten asphaltic material, which is heated to a temperature of about 150° C., 90 for a period of from three to four hours. 95

The action which takes place under this 100 procedure is believed to be as follows: It is well known that paraffin or similar materials will penetrate the pores of wood rather readily, whereas a heavier material, such as asphalt, will penetrate very slightly, due to the higher viscosity thereof. By first impregnating the wood with paraffin and then subjecting the same to higher temperatures in a bath of asphalt, the paraffin will be 105 partially displaced at the higher temperatures by the heavier, more viscous material which is drawn into the individual cells of the wood by reason of the partial vacuum created therein. By this treatment, I am 110

enabled to produce a much greater penetration of asphaltic material than hitherto, many tests showing a penetration of from three-eighths to one-half inch, whereas, by former methods, the asphaltic material did not generally penetrate more than one-eighth inch.

This process of impregnating wood gives a high dielectric strength thereto without any loss of mechanical strength and simultaneously renders the wood moisture and weather-proof. The heat of the sun has practically no effect upon the impregnating materials which are not evaporated under the action of the direct rays of the sun.

By reducing the moisture content of the material to be impregnated to ten to twelve per cent, I remove a large proportion of the water in the wood, thus rendering it easier for the paraffin to penetrate the pores, which still remain open. If the moisture content should be reduced to a substantial degree below ten per cent, most, or many, of the pores would become closed and would offer relatively great resistance to the penetration of the paraffin.

The central portion of the insulator, being filled with paraffin, is rendered moisture-proof so that, even if the outer layer of asphalt is defective, moisture will still be unable to enter the wood and impair the insulating properties thereof. The asphaltic material along the outer portion also aids in rendering the wood moisture-proof and water-resistant and, being non-volatile, remains permanently in place, preventing the relatively volatile paraffin from escaping.

Wood impregnated by this method shows great resistance to electrical strains. For instance, several impregnated sticks of wood were tested by applying 100,000 volts between the ends thereof for about five minutes. The voltage was then raised to 300,000 with no flash-over or injury to the wood. The sticks were then immersed in water for forty-eight hours, being weighed before and after immersion, and showed less than one per cent absorption of moisture. The sticks, after removal from the water, were surface dried, after which a potential of 100,000 volts was applied for five minutes. The voltage was then gradually increased and it was found that the discharge flashed over at somewhat above 250,000 volts. Upon examination, the wood was found not to be injured in the least. The sticks were then

subjected to varying voltages while a shower of spray was caused to fall on the sticks, which were placed at angles of about 15°. Arcing began when the voltage reached 90,000 to 95,000 and the discharge flashed over at 175,000 to 185,000 volts. A mechanical-strength test showed no deterioration whatsoever.

It is obvious that materials other than paraffin, such as natural or artificial waxes, greases, fats, gums of low viscosity, etc., which have great penetrating and insulating properties, may be used. The asphalt may be replaced by tars, pitches, heavy gums, cresols, and the like, which are insoluble in water and are non-volatile and have insulating properties. It is also apparent that various other changes may be made in practising my invention, all of which are considered to be within the scope thereof.

I claim as my invention:

1. A method of preparing an impregnated body of wood which comprises drying the wood to a moisture content of 10 to 12%, impregnating the wood in a bath of paraffin at an elevated temperature and subsequently heating said impregnated wood in a bath of asphaltic material at a higher temperature.

2. A method of impregnating wood which consists in impregnating the same with a wax at an elevated temperature, and subsequently subjecting the same to impregnation with a gummy material at a higher temperature.

3. A method of impregnating wood which consists in drying the same to reduce its moisture content to 10 to 12 per cent, then impregnating the same with paraffin for five to six hours at a maximum temperature of 130° C., and subsequently subjecting the same to impregnation with asphalt for three or four hours at a temperature of about 150° C.

4. Wood, the inner portions of which are impregnated with paraffin and the outer layers of which are impregnated with asphalt.

5. A wood strain-insulator having its interior impregnated with paraffin and its exterior impregnated with asphalt.

In testimony whereof, I have hereunto subscribed my name this 7th day of December 1920.

OTHO V. STEWART.